# EUROPEAN PATENT APPLICATION

(11) **EP 1 918 502 A1**
(43) Date of publication of application: **07.05.2008**
(21) Application number: 06076943.7
(22) Date of filing: 27.10.2006
(51) Int. Cl.: E06B 5/10

(54) **Method for armouring a window**

(71) Applicant: Nederlandse Organisatie voor toegepast-natuurwetenschappelijk Onderzoek TNO, 2628 VK Delft (NL)
(72) Inventor: Broos, Johannes Pieter Frans, 2691 RH 's Gravenzande (NL); Carton, Erik Peter, 2497 AA Den Haag (NL)
(74) Representative: van Loon, C.J.J.

(57) **Abstract**

The invention relates to a method for armouring a window of an existing object comprising applying a transparent polymer layer to a surface of the window. The layer is usually applied to a surface facing the inside of the object. In particular, the invention may be employed to a conventional glazing of a building or vehicle.

## Description

The invention relates to a method for armouring a window of an existing object.

Transparent armour materials with antiballistic properties are usually made of multiple layers of transparent material having a hard frangible flat face plate backed by one or more transparent tough resilient plates, bonded together by a suitable transparent adhesive. Such armour is for instance described in United States Statutory Invention Registration H1567 (application number 667,624). Another laminated transparent armour is described in United States Statutory Invention Registration H1519 (application number 522,788).

In the art windows with an antiballistic function comprise a special glass, having a high resistance against high velocity impact against bullets and/or other missiles.

The use of special glasses is expensive. Also, armour glass plates are usually flat as these tend to be difficult to shape in curved forms, for practical reasons. Further, these glasses tend to have a large thickness, which makes windows composed thereof heavy. This may require special measures to be taken in order to support the window in the object, e.g. fortification of hinges, grooves or the frame. This may further increase the weight of the object.

Furthermore, in order to protect windows in an existing object against the impact of a projectile such as a bullet, it is not only expensive but also laborious to have to replace existing windows with such material. Further, it is practically impossible to shoot from the protected side of the window.

It is an object of the present invention to provide a novel method for armouring a window of an object.

It is in particular an object to provide a method that can overcome one or more of the above identified drawbacks.

One or more objects which may be solved in accordance with the invention may be derived from the description herein below.

The inventors have realised that it is possible to improve an antiballistic property of a window in an existing object, in particular a window, such as ordinary windowpane or ordinary car glass. They have further realised that this is possible by *in situ* applying a layer of a specific material to the window.

Accordingly, the present invention relates to a method for armouring a window of an existing object comprising applying a transparent polymer layer to a surface of the window.

In particular, the present invention relates to a method for armouring a window of an existing object comprising applying a transparent polymer layer to a surface of the window, said polymer layer having a thickness of at least 5 mm and a strength of at least 2 MPa.

In particular, the transparent polymer layer is applied to a surface of the window opposite to the surface from which a ballistic threat can generally be expected. Accordingly, usually an inner surface of the window in the object is provided with the polymer layer. In an embodiment, it is advantageous that the invention allows a subject inside the object, who is protected by the window, to shoot through the window, whilst maintaining some level of protection, as a bullet shot by the subject first penetrates through the polymer and thereafter through the glass. On the other hand, a bullet or the like impacting the window from the other side will generally be stopped by the armoured window.

The glass and the polymer layer may act synergistically with respect to an antiballistic property. It is contemplated that the polymer allows the glass to have a better antiballistic performance. The polymer layer supports and/or strengthen the glass. Thus the anti-ballistic protection provided by the glass is improved, also if polymer layer and/or the glass as such do not show a considerable ballistic protection.

The object may in particular be a building - such as an embassy or a bank - or a transportation device, in particular a vehicle, boat or plane.

The window provided with the polymer layer is transparent, preferably at least as transparent as water. The term "transparent" is generally understood in the art. It will be understood that transparency is to some extent dependent upon the thickness of the armour. In particular a material, such as the armour/pellet/matrix/backing material, is considered transparent if the luminous transmission is 85 % or more and the haze is 5 % or less.

The window may be a flat or curved panel, a screen, a canopy, a windshield, a visor, a dome or the like. It is advantageous that the method of the invention can also easily be employed to a curved surface. For instance, armoured transportation devices, such as armoured cars, with special glass windows normally have flat windows. This makes the vehicles easily recognisable as armoured vehicles, which may cause aggression to adversaries of the people inside the vehicle in some circumstances, e.g. during peace keeping operations. When applied to a normal window, it is less noticeable that the vehicle is provided with a protection against an impact by a projectile.

It is advantageous to improve an antiballistic property of the window in accordance with the invention by applying the polymer layer without detaching the window from the object. The layer can easily be applied whilst the window remains part of the object.

It has been found that also an antiballistic property of an ordinary window, made of a standard glass, for instance ordinary car glass can be improved in accordance with the invention. E.g. as shown in Example 1, a windscreen of a truck can be made resistant to the impact of projectiles from hand-guns, e.g. 9 mm bullets and fragments of a bomb, e.g. of about 1 g weight impacting at a velocity of about 1300 m/s.

The inventors have found that it is particularly advantageous with respect to improving the multi-hit capacity of the armour by providing the armour with a visco-elastic material. For improving multi-hit capacity, the visco-elastic relaxation time, preferably should be in the range of 10⁻⁹ - 10⁻¹ [s]. The hardness preferably is 70 - 100 Shore A

The polymer layer may in particular comprise one or more polymers selected from the group consisting of transparent acrylonitrile-butadiene-styrene; transparent acetal resins; transparent cellulose derivatives, in particular such cellulose esters, such as cellulose acetate, cellulose butyrate, cellulose propionate, cellulose triacetate and alkyl celluloses, such as ethyl cellulose; transparent acrylics, transparent allyl resins; transparent polyethers, in particular such chlorinated polyethers; transparent fluoroplastics; transparent melamines; transparent polyamides (nylon; transparent parylene polymers; transparent phenolics; transparent phenoxy resins; transparent polybutylene, transparent polycarbonates; transparent polyesters; transparent polyethylenes; transparent polypropylenes; transparent polyphenylenes; transparent polystyrenes, transparent polyurethanes; transparent polysulphones; transparent polyvinyl alcohols; transparent polyvinyl fluorides; transparent polyvinyl butyrals; transparent polyvinylidene chlorides, transparent silicones; transparent styrene acrylonitrides; transparent styrene butadiene; transparent polyvinylchlorides; including transparent copolymers of any of these.

Preferably the polymer layer comprises a polymer selected from the group consisting of transparent polyurethanes, transparent silicones, transparent polyvinylchlorides and transparent polycarbonates.

Particularly good results have been achieved with a transparent polyurethane, in particular with respect to transparency, (visco)-elastic properties and/or adherence to the surface of the window.

Suitable polyurethane resins for providing the polymer layer are commercially available. Examples thereof include: Castable transparant Polyurethane resin (PUR, such as ClearFlex hardness Shore A between 50 and 90, manufacturer Smooth-On, 2000 Saint John Street, Easton, PA 18042); MB International 438 PU; MB International Poly A80; Permapur RD 3505; Simula: SIM 2025, SIM 2003.

The mixture for providing the polymer layer preferably has a low viscosity, in particular a viscosity (at 25 °C) of 100 Pa.s or less.

The potlife of the mixture is the maximum period of time wherein the resin can be processed without substantially influencing the end result. The Potlife preferably is relatively long, in particular at least 25 min, e.g. 20-40 min.

After curing, the polymer layer preferably meets one or more of the following criteria:
- shrinkage (compared to uncured resin): 0.3 % or less, in particular 0.15-0.3%.
- elongation until rupture: at least 100 %, in particular 175-500 %
- tensile strength: at least 2 MPa, in particular 2-20 MPa.
- tear strength: at least 0.2 MPa, in particular 0.2-2 MPa.
- hardness: at least Shore A 50, in particular Shore A 50 - 95.
- Glassy (dynamic, 1 Hz) Young's modulus: about 2700 MPa.
- Rubber (dynamic, 1 Hz) Young's modulus: about 4.5 MPa
- glass transition temperature about 20 ± 5 °C.
- a relaxation curve as measured by the method described in "C van 't Hof, Mechanical Characterization and Modeling of Curing Thermosets, PhD thesis Delft University of Technology, 2005, essentially corresponding to the curve shown in Figure 1.

Tear strength may be determined according to ISO 34, Hardness according to ISO 868, parameters obtainable by a tensile test according to ISO 35.

Optionally, the polymer layer comprises one or more additives in order to alter a mechanical property, adherence to the surface of the window and/or transparency.

The window may in principle be composed of any transparent material suitable for a window. Usually it is a glass material suitable for a normal use in a particular object, such as normal glazing for a building.

In particular, the window may be composed of a glass selected from tempered glass, layered glass, or a normal glazing for a vehicle or a building.

The thickness of the window to be armoured may be within a usual range for a window in the specific object. In general, the thickness may be in the range of 2 to 15 mm. In particular, the thickness of a window in a vehicle may be 3 to 7 mm. The thickness of a window in a building may in particular be in the range of 4 to 12 mm.

Preferably, the surface of the window may be cleaned before applying the layer. It is in particular desired to remove dust and/or grease, if present on the surface.

The polymer layer is preferably at least applied at a surface opposite the surface from which a thread is expected, so usually to a surface of the window facing the inside of the object. Thus, a projectile impacting on the window would first hit the surface of the window opposite of the polymer layer, deform the projectile, and locally tear or even shatter at least to some extent. The polymer layer at the other surface is particular suitable to substantially reduce the degree of tearing or shattering and/or avoiding spreading of fragments of the glass, which is also relevant for blast protection.

The polymer layer may be applied while the material for forming the layer is fluid, e.g. by brushing or casting, after which the material is allowed to solidify. Solidification may be carried out in a manner known in the art *per* se, for the specific material. Specific material properties, such as elasticity or visco-elasticity, ductility etc. may be controlled by the choice of components and ratio from which the layer is composed, such as chemical structure and average polymer weight of the polymer and/or the presence of a cross-linking agent.

In order to avoid flowing of the fluid polymer or polymer composition over or from the surface before it has sufficiently solidified, the fluid polymer may be held in between the surface of the window and a rigid support, e.g. a glass or metal plate. In order to avoid sticking of the polymer layer to the support, the support may be pre-treated with an anti-adhesive for the polymer layer, generally known as release agent, e.g. polytetrafluorethylene (such as Teflon®). After sufficient solidification of the polymer layer, the support is removed.

For ease of application, it is preferred to first prepare a polymer sheet with the desired thickness and properties which is thereafter adhered to the window. The sheet can be prepared on a large scale in a factory and thereafter anywhere applied to the window of the object. Thus, the person actually applying the polymer layer to the window needs not to be skilled to prepare polymer layers from base materials. Also, this it is easier to control the thickness of the polymer layer and its properties such as mechanical properties and transparency.

The sheet may be adhered to the surface of the window using a suitable adhesive, for instance a polyurethane adhesive and/or a polyvinylbutyral adhesive.

The thickness of the layer can be chosen within wide limits, depending upon the mechanical properties of the layer, the desired improvement in an antiballistic property, and practical reasons such as the maximum possible or desired thickness of the window including polymer layer in view of aesthetic considerations and/or the functioning of the object.

For improving an antiballistic property, the thickness of the layer is usually at least 5 mm, preferably at least 10 mm, more preferably at least 15 mm. Particular results have been achieved with a layer having a thickness of 20 mm or more.

For practical reasons, such as mass limitation, the thickness is generally 40 mm or less, preferably 30 or less, in particular in a transport, such as a car, a bus, a truck or an aircraft.

If desired, the side of the polymer layer opposite to the window to which it is attached, may be provided with a transparent plastic sheet to improve smoothness of the layer, in particular in case the polymer layer is sticky and/or to protect the layer from being damaged during normal use. Such sheet can be relatively thin, in particular 1 mm or less, e.g. 0.1-1 mm. A particularly suitable sheet is a transparent polycarbonate sheet.

The invention will now be illustrated by the following examples.

### Example 1: PUR Casting process

The inner surface of the windscreen (a layered glass construction with a total thickness of 6.6 mm) was cleaned using water and soap and finally with acetone.

Then the area to be protected was surrounded by a 4 cm high strip of polyethylene which was watertight connected to the glass surface (by waterproof tape or an elastomeric strip).

The right amount of components A (polyol) and B (isocyanates) of the Smooth-on product Clear Flex were mixed in the required mass ratio (100:175) by mechanical stirring in a mixing container (polyethylene). After 5 minutes of active mixing the container is vacuumized for 2 minutes in order to remove entrapped air from the mixture.

Then the mixture was gently applied onto the glass surface in a corner of the area to be covered. Then the mixture reacted and hardened as well as bonded to the glass surface, the hardness of the PUR layer was measured as Shore A 75.

### Example 2: PUR plate fabrication and adhesion process

A simple rectangular watertight container or box was made from aluminum plate material (size 200 x 300 x 40 mm), then the die was internally covered with PE-plates. PE does not adhere to polyurethane resin (PUR).

Enough of the PU mixture (components A and B in the required mass ratio) was made in the same way as described above and poored into the PE covered die.

The mixture reacted and cured in the container in the form of a flat plate. The container walls were removed and the PUR plate was taken away from it.

The inner surface of a car door window was cleaned using water, soap and acetone. The side window of a car exists of a single layer of tempered glass. Its thickness was 4.9 mm. A small amount of PUR mixture was made in the right amount of components A (polyol) and B (isocyanates) of the Smooth-on product Clear Flex are mixed in the required mass ratio (100:150) by mechanical stirring in a plastic cup.

After vacuumizing this mixture, a small amount is poored on the inner glass surface. The PUR plate was carefully layed on top of the horizontal positioned glass, taking care that no air bubbles were entrapped between the glass and the PUR. The PUR plate was mechanically pressed onto the glass using a mass divided over its surface (using a powder inside a bag) .

After 12-24 hours the resin cured and the PUR-plate was well bonded to the glass.

### Ballistic testing

The ballistic tests on the flat glass objects with and without the PUR backing layers have been performed using steel fragment simulating projectiles (FSP) with a mass of 1.1 gram. Its impact velocity on the glass layer could be controlled. The V50 corresponds to a velocity of the FSP that upon perpendicular impact to the target has a 50% chance to penetrate the target material.

First the windscreen was tested without a PUR backing layer and the V50 of the 1.1 gram FSP was determined to be 300 m/s. The same windscreen was shot using a fire-arm projectile (9mm Ball DM41) with an impact velocity of 427 m/s, which easily penetrated the glass as its residual velocity was still high (339 m/s).

Then the area of the windscreen that had a 20 mm thick PUR backing layer (shore A 75) was tested.

The V50 of the polymer backed windscreen was increased to 1300 m/s using the 1.1 gram FSP. Also this protected area was shot using the 9 mm Ball DM 41 bullet with an impact velocity of 433 m/s. The bullet did not penetrate the target and was recovered heavily deformed at the glass/polymer interface. The glass layer was heavily damaged in an area with a radius of 3 cm around the impact site. Also some longer cracks were visible in one layer of the (two-layered) glass. The polymer layer was not broken or fractured and was still transparent.

The ballistic properties of the car door window were measured by V50 determination using the 1.1 gram FSP as well.

The unprotected tempered glass has a V50 of about 240 m/s (less then the windscreen due to its reduced glass thickness). Due to its internal stress (which is normal in tempered glass) the glass fragmented totally in many small pieces.

The PUR backed car door window using adhesion of the PUR-layer showed an increased ballistic protection of its V50 value to 940 m/s. Also in this case did the glass fragment totally, however the fragments remained adhered to the PUR backing layer. This allowed the window to stop also following (multiple) FSP impacts.

## Claims

1. Method for armouring a window of an existing object comprising applying a transparent polymer layer to a surface of the window, wherein the strength of the polymer layer is at least 2 MPa and the thickness of the polymer layer is at least 5 mm.

2. Method according to claim 1, wherein the layer is applied to a surface facing the inside of the object.

3. Method according to claim 1 or 2, wherein a transparent ductile polymer sheet is adhered to the surface.

4. Method according to any one of the preceding claims, wherein the polymer layer is an elastic or visco-elastic layer.

5. Method according to claim 1 or 2, wherein a fluid polymer or fluid polymer composition is applied to the surface, which polymer or polymer composition is thereafter allowed to cure.

6. Method according to claim 5, wherein after applying the polymer or polymer composition, a transparent sheet is applied to the surface of the polymer layer.

7. Method according to any one of the preceding claims, wherein the ductile polymer layer comprises a visco-elastic polymer.

8. Method according to any one of the preceding claims, wherein the polymer layer comprises one or more polymers selected from transparent acrylonitrile-butadiene-styrene; transparent acetal resins; transparent cellulose derivatives, in particular such cellulose esters, such as cellulose acetate, cellulose butyrate, cellulose propionate, cellulose triacetate and alkyl celluloses, such as ethyl cellulose; transparent acrylics, transparent allyl resins; transparent polyethers, in particular such chlorinated polyethers; transparent fluoroplastics; transparent melamines; transparent polyamides (nylon; transparent parylene poloymers; transparent phenolics; transparent phenoxy resins; transparent polybutylene, transparent polycarbonates; transparent polyesters; transparent polyethylenes; transparent polypropylenes; transparent polyphenylenes; transparent polystyrenes, transparent polyurethanes; transparent polysulphones; transparent polyvinyl alcohols; transparent polyvinyl fluorides; transparent polyvinyl butyrals; transparent polyvinylidene chlorides, transparent silicones; transparent styrene acrylonitride; transparent styrene butadienes; transparent polyvinylchlorides; including transparent copolymers of any of these.

9. Method according to any one of the preceding claims, wherein the window is composed of a glass selected from the group consisting of single layer tempered or single-layer untempered glass, layered glass, vehicle glazings, boat glazings, plane glazings, and building glazings

10. Method according to any one of the preceding claims, wherein the object is selected from buildings, counters and transports, in particular from vehicles, boats, planes, banks and embassies.
